# EUROPEAN PATENT SPECIFICATION

(11) **EP 1 943 314 B1**
(45) Date of publication and mention of the grant of the patent: **19.08.2015**
(21) Application number: 06803035.2
(22) Date of filing: 06.09.2006
(51) Int. Cl.: C09D 4/00, C09D 183/08, C09J 5/02, C08K 5/548, C08K 5/544, C23C 22/02, B05D 1/36

(54) **METHOD OF APPLYING SILANE COATING TO METAL COMPOSITION**
VERFAHREN ZUR APPLIZIERUNG EINER SILANBESCHICHTUNG AUF EINER METALLZUSAMMENSETZUNG
PROCEDE D'APPLICATION D'UN REVETEMENT DE SILANE SUR UNE COMPOSITION METALLIQUE

(30) Priority: 09.09.2005 US 715474 P; 02.03.2006 US 366235
(43) Date of publication of application: 16.07.2008
(73) Proprietor: UNIVERSITY OF CINCINNATI, Cincinnati, OH 45221-0623 (US); ECOSIL TECHNOLOGIES LLC, Fairfield, OH 45014 (US)
(72) Inventor: SMITH, Charles, Conway, AR 72034 (US); SORENSON, Max, Salt Lake City, UT 84121 (US); VAN OOIJ, William, J., Fairfield, OH 45014 (US); NOOKALA, Ramakrishna, Greenville, SC 29615 (US); WILLIAMS, Kevin, Benton, AR 72015 (US)
(74) Representative: Findlay, Alice Rosemary
(86) International application number: PCT/US2006/034705
(87) International publication number: WO 2007/030532

(56) References cited:
- WO-A-00/38844
- WO-A1-00/39356
- WO-A2-2005/035634

## Description

### RELATED APPLICATIONS

This application is related to provisional application 60/715,424, the disclosure of which is hereby incorporated by reference.

### BACKGROUND OF THE INVENTION

Silanes are applied to metal surfaces for several purposes including corrosion resistance and adhesion promotion. As an example, steel tire cord must adhere to the rubber in order to function properly. Steel does not bond well to rubber. To improve adhesion, the steel tire cord has been coated with a layer of brass. During the vulcanization process, the rubber forms a chemical bond with the brass. This rubber/metal bond is formed only with sulfur vulcanized rubber which requires a relatively high sulfur level, greater than 4 phr, as well as certain accelerators, i.e., a delayed action sulfonamide and cobalt in the form of cobalt naphthenate to achieve proper cure and good adhesion, as well as zinc oxide. The cobalt improves the stability of the rubber/brass bond. However, it also has a negative effect on the stability of the rubber network in that it accelerates reversion in the presence of oxygen at elevated temperatures. The increased sulfur and cobalt are believed to be necessary in order to achieve a satisfactory bond between the tire cord and the rubber.

It has been proposed to treat tire cord with various silane compositions in order to improve adhesion. This is disclosed, for example, in van Ooij U.S. patent 6,416,869; U.S. patent 6,756,079; and U.S. patent6,919,469. The processes disclosed in these patents have various problems. One primary problem is the efficient application of the silane onto the tire cord. Some of these applications require that the silane be baked onto the tire cord in order for adequate adhesion.

Silane coatings are also applied to other forms of metals. They may be applied in aqueous solution, or suspension, or dissolved in a volatile solvent.

WO00/38844 discloses a method for applying a silane onto a metal surface. In one example a mixture of 20% process lubricant, 77.6% water and aqueous silane is applied. The process lubricant is about 6 to 12% mineral oil with emulsifiers in water.

### SUMMARY OF THE INVENTION

The present invention provides a method of applying a silane coating onto a metal substrate comprising contacting said metal substrate with an oil mixture wherein said oil mixture comprises at least 80% by weight oil and 0.5% to 10% organofunctional silane by weight, and wherein the oil is selected from the group comprising naphthenic lubricating oils, paraffinic lubricating oils, polyglycols, animal based lubricating oils, vegetable based lubricating oils and synthetic lubricants comprising dibasic acid esters, chlorofluorocarbons, silicone oils, neopentyl polyol esters and polyphenyl ethers.

The invention also provides a coating composition comprising at least 80% by weight oil and 0.5% to 10% organofunctional silane by weight, and wherein the oil is selected from the group comprising naphthenic oils, paraffinic oils, polyglycols, dibasic acid esters, chlorofluorocarbons, silicone oils, neopentyl polyol esters and polyphenyl ethers.

The present invention is premised on the realization that metal such as tire cord can be coated with a silane coating by running the metal through an oil bath containing a small percentage of sliane. Excess material is simply wiped off using an air wipe or other similar device. With respect to coating tire cord, this is advantageous because the tire cord normally must pass through an oil bath during processing.

Any organo-functional silane can be employed. Such silanes are known to Improve adhesion and prevent corrosion. For tire cords. the silane can be any organosillane that Improves rubber/metal adhesion. These can include, for example, vlnylsllanes, amlnosilanes, polysulfidesilanes, as well as blends of organosilanes. For sulfur cure rubber systems the silane will be a blend of an amino silane and a polysulfide silane.

This, In turn, allows the rubber formulation, in particular the sklm rubber formulation, to have less sulfur and no cobalt or zinc oxide, thereby Improving the performance characteristics, such as heat aging, of the formed tire. This also significantly reduces the cost of the rubber formulation.

This method can be used to coat any type of metal, Including brass, aluminum, steel and galvanized metal.

The objects and advantages of the present invention will be further appreciated In light of the following detailed description and drawing, In which:

### BRIEF DESCRIPTION OF THE DRAWINGS

The Figure Is a diagrammatic deplotion, partially broken away, of the apparatus used to coat tire cord.

### DETAILED DESCRIPTION OF THE INVENTION

According to the present invention, metal is coated with an organofunctional silane utilizing an oil bath containing the silane. The organosilane, can be any orgenosilane. These may be added to provide corrosion resistance or as an adhesion promoter, in particular a metal-rubber adhesion promoter. In a preferred embodiment, the metal Is a wire, and in particular steel or brass coated steel tire cord. The rubber can be any rubber that incorporates metal such as tires and conveyor belts.

Typical organofunctional silanes used in these applications include vinyl silanes, aminosilanes, and polysulfidesilanes, as well as mixtures thereof. Such silanes are disclosed in U.S. patent 6,416,869; U.S. patent 6,756,079; PCT application WO2004/009717; pending application U.S. 2005/0058843; and U.S. patent 6,919,469.

One preferred silane coating composition for sulfur cured rubber systems is a blend of a bis-silyl amino silane and a bis-silyl polysulfur silane, with the ratio of bis-silyl amino silane to bis-silyl polysulfur silane from about 1:10 to about 10:1, preferably 1:3, by weight.

The preferred bis-silyl aminosilanes which may be employed In the present Invention have two trisubstituted silyl groups, wherein the substituents are individually chosen from the group consisting of alkoxy, aryloxy and acyloxy. Thus, these bis-silyl aminosilanes have the general structure: wherein each R¹ is chosen from the group consisting of: C₁-C₂₄ alkyl (preferably C₁-C₆ alkyl), and C₂-C₂₄ acyl (preferably C₂-C₄ acyl). Each R¹ may be the same or different, however, In the hydrolyzed silane solutions, at least a portion (and preferably all or substantially all) of the R¹ groups are replaced by a hydrogen atom. Preferably, each R¹ is individually chosen from the group consisting of: ethyl, methyl, propyl, iso-propyl, butyl, iso-butyl, sec-butyl, ter-butyl and acetyl.

Each R² in the aminosilane(s) may be a substituted or unsubstituted aliphatic group, or a substituted or unsubstituted aromatic group, and each R² may be the same of different. Preferably, each R² is chosen from the group consisting of: C₁-C₁₀ alkylene, C₁-C₁₀ alkenylene, arylene, and alkylarylene. More preferably, each R² is a C₁-C₁₀ alkylene (particularly propylene).
X may be: wherein each R³ may be a hydrogen, a substituted or unsubstituted aliphatic group, or a substituted or unsubstituted aromatic group, and each R³ may be the same or different. Preferably, each R³ is chosen from the group consisting of hydrogen, C₁-C₆ alkyl and C₁-C₆ alkenyl. More preferably, each R³ is a hydrogen atom.

Finally, R⁴ in the aminosilane(s) may be a substituted or unsubstituted aliphatic group, or a substituted or unsubstituted aromatic group. Preferably, R⁴ is chosen from the group consisting of: C₁-C₁₀ alkylene, C₁-C₁₀ alkenylene, arylene, and alkylarylene. More preferably, R⁴ is a C₁-C₁₀ alkylene (particularly ethylene).

Exemplary preferred bis-silyl aminosilanes which may be used in the present invention include bis-(trimethoxysilylpropyl) amine (which is sold under the tradename Silquest® A-1170 by GE Silicones); and bis-(trimethoxysilylpropyl)ethylene diamine.

The preferred bis-silyl polysulfur silanes which may be employed in the present invention include: wherein each R¹ is as described before. In the hydrolyzed silane solutions of the present invention, at least a portion (and preferably all or substantially all) of the R¹ groups are replaced by a hydrogen atom. Z is -Q-Sₓ-Q-, wherein each Q is an aliphatic (saturated or unsaturated) or aromatic group, and x is an integer of from 2 to 10. Q within the bis-functional polysulfur silane can be the same or different. In a preferred embodiment, each Q is individually chosen from the group consisting of: C₁-C₆ alkyl (linear or branched), C₁-C₆ alkenyl (linear or branched), C₁-C₆ alkyl substituted with one or more amino groups, C₁-C₆ alkenyl substituted with one or more amino groups, benzyl, and benzyl substituted with C₁-C₆ alkyl.

Particularly preferred bis-silyl polysulfur silanes include bis-(triethoxysilylpropyl) sulfides having 2 to 10 sulfur atoms. Such compounds have the following formula: wherein x is an integer of from 2 to 10. One particularly preferred compound is bis-(triethoxysilylpropyl) tetrasulfide (also referred to as bis-(triethoxysilylpropyl) sulfane, or "TESPT"). Commercially-available forms of TESPT (such as Silquest® A-1289, available from GE Silicones), however, are actually mixtures of bis-(triethoxysilylpropyl) sulfides having 2 to 10 sulfur atoms. In other words, these commercially-available forms of TESPT have a distribution of sulfide chain lengths, with the S₃ and S₄ sulfides predominating.

Silanes can be either hydrolyzed or unhydrolyzed, and can be utilized in combination with an aqueous resin dispersion. Typically, the silanes are not hydrolyzed when combined with the resin dispersion, as well as when added directly to the oil bath as described below. However, the silanes tend to hydrolyze through exposure to air.

For use in the present invention a variety of water dispersible resins can be employed including epoxy resins, novolac resins, acrylate resins, and polyurethane resins. In addition to the water dispersible resins, neat resins can also be used that are compatible with the oil and the selected silane. The water borne dispersion of polymeric resin may also include a certain percentage by volume of an organic solvent, such as an alcohol (e.g. ethanol), as well as surfactants used to keep the resin in solution or dispersed in the water. In one example, the dispersion includes about 50% by volume of an n-butoxy ethanol.

The resin dispersion may be purchased commercially and can include, for example, Epi-rez 5522-WY-55, a 55% solids dispersion of a modified polyfunctional epoxy resin in water and 2-propoxy ethanol, (available from Resolution Performance LLC), or Epi-rez WD 510, a water reducible epoxy resin, or ECO CRYL 9790, an aqueous acrylic with 42% solid dispersed in 45% water, 7% 2-propoxy ethanol, 3% xylene and 3% ethanamine.

The silane is applied to the metal In an oil bath. If silane is used without resin the silane is added directly to the oil bath. The concentration of the silane should be from about .5% to about 10% by weight, preferably about 2%, with 6% most preferred. The oil should comprise 80% or more of the bath (by weight) with at least 95% preferred. If the silane is combined with an aqueous dispersion of a resin, the ratio of resin dispersion (50-55 active) to silane by weight should be from about 1:5 to about 5:1, with 1:1 preferred. It is generally desirable to minimize the amount of resin, using only enough to insure the silane is dispersed in the mixture. If added, the silane is mixed with the resin dispersion, sufficient dispersion is added to the oil bath to provide 5-10% by weight silane in the bath, with 6% by weight preferred.

The oil is a non VOC lubricating oil and can be any mineral, animal or vegetable based lubricating oil. Oil includes synthetic lubricants such as polyglycols, dibasic acid esters, chlorofluoro carbons, silicone oils, neopentyl polyol esters, and polyphenyl ethers. Preferably, the oil will be a mineral oil, such as a paraffinic or naphthenic lubricating oil, having a viscosity such that it flows at application temperature. Any oil which can be used in a tire cord manufacturing process can be used in the present invention. One such oil is a heavily hydrotreated naphthenic having a viscosity of 60 SUS @ 100°F CAS 647-52-5.

Prior to coating the metal in the oil bath, the metal should be cleaned with an acid or alkaline cleaner and rinsed with deionized water, preferably, an alkaline cleaner. The silane oil mixture can be applied to the metal surface by any common method such as spraying, brushing, emersion coating, curtain coating, and the like.

When the metal is wire, such as tire cord, it can be coated with an apparatus such as that shown in the Figure. The Figure shows an exemplary coating apparatus 10 adapted to coat tire cord 12 with oil 17 containing the silane. As shown, the apparatus 10 is a trough which is divided by barrier 11 into first and second sections 13 and 15. First section 13 includes first and second grooved rollers 14 and 16. The cord 12 runs back and forth in grooves in rollers 14 and 16 and is thus repeatedly submersed in the oil 17 in first section 13. The cord 12 moving in the direction of arrows 26 then passes through an air wipe 18 which forces off excess oil and coating material. This excess is then taken from second section 15 of apparatus 10 and redirected through line 20 and redeposited back on roller 14 into the first section 13 of the coating trough 10.

The temperature of the oil bath will generally be about room temperature (50-120°F), but can be raised up to the boiling point of the oil. The cord should be in oil for .1 to 10 seconds, preferably 1-2 seconds. This is controlled by controlling the path through the oil as well as the speed of cord 12.

After being coated, the cord is simply rolled onto a spool and then can subsequently be used to form belting for tires, conveyer belts, and the like. Typical rubber formulations are disclosed in U.S. patent 6,919,469, the disclosure of which is incorporated herein by reference.

To test the rubber adhesion between the silane coated cord and sulfur cured rubber, a series of tests were performed. These tests used hydrolyzed and unhydrolyzed silanes and used silanes with and without a resin coating.
Materials used: Tire cords, amino silane A1170, Sulfane A1289, Epi-rez 3510 W-60, Epi-rez WD 510, Lubesnap 60 lubricant.
Surface treatment: 1 M NaOH dip, air dry, DI rinse, air dry, 1 M NaOH dip, air dry, DI rinse, air dry.
Rubber used: The Test compounds include a typical tire rubber formulation that has excellent adhesion to brass incorporating cobalt naphthenate and a compound used for test purposes that has no adhesion to brass, i.e., without cobalt naphthenate.
Vulcanization parameters: 172°C for 16 minutes at 43 kg/m².
Analytical technique: Adhesion pull out testing in tension.

Epi-rez WD 510 contains 100% solid with greater than 90% bisphenol A epoxy resin and less than 10% polymeric dispersant. Epi-rez 3510 W-60 is an aqueous dispersion of bisphenol A epoxy resin, which contains 61% solid in water. The below matrix describes the physical constituents of the hydrolyzed silane mixtures.

**Table 1**

| **Description of the hydrolyzed silanes** | | | | |
|---|---|---|---|---|
| Silane mixture | Neat A1170 (ml) | Neat A1289 (ml) | Acetone (ml) | Water (ml) |
| 10% A1170 | 10 | 0 | 0 | 90 |
| 62.5% A1289 | 0 | 50 | 15 | 15 |
| 43.5% A1289 | 0 | 50 | 50 | 15 |

The following tests were conducted to study the difference in performance between the oil based and water based resin silane mixtures.

The below listed values are measured on a 100g total weight basis. The wires were cleaned as previously described. A 1:3 ratio was maintained between A1170 and A1289. The wires after being cleaned were coated with the above silane mixtures and cured in rubber and tested under tension for adhesion.

**Table 2**

| **Description of the silane mixtures** | | | | | | |
|---|---|---|---|---|---|---|
| Silane mixture | A1170 (g) | A1289 (g) | Epi-rez 3510 W-60 (g) | Lubricant | Water | Drying °/minutes |
| A | 0.25 | 0.75 | 1.0 | NA | 98 | 105/3 |
| B | 0.25 | 0.75 | 1.0 | 98 | NA | NA |
| C | 0.25 (10%) | 0.75 (43.5%) | 1.0 | 98 | NA | NA |
| D | 0.25 (10%) | 0.75 (62.5%) | 1.0 | 98 | NA | NA |
| E | 0.25 | 0.75 | 1.0 | 98 | NA | 105/3 |
| F | 0.25 (10%) | 0.75 (43.4%) | 1.0 | 98 | NA | 105/3 |
| G | 0.25 (10%) | 0.75 (62.5%) | 1.0 | 98 | NA | 105/3 |

The pull out force for the respective samples and an uncoated control were as follows:

| | |
|---|---|
| Control | 12.5 kg |
| A | 17.0 kg |
| B | 21.0 kg |
| C | 21.0 kg |
| D | 17.0 kg |
| E | 27.3 kg |
| F | 22.0 kg |
| G | 20.5 kg |

The matrix listed below assesses the effect of cleaning and drying on the oil based WD 510 resin silane system. The neat silane concentration was 20% by weight and the ratio of A1170 to A1289 is 1:3. Equal parts of A1170 and WD 510 were added. The tire cords were cured in the experimental rubber and tested under tension for adhesion.

**Table 3**

| | Dried | Not Dried |
|---|---|---|
| Cleaned | 1 | 2 |
| Not cleaned | 3 | 4 |

The oil based silane resin mixture B works better than the water based resin silane mixture A. Both these mixtures offered the same rubber coverage.

Silane mixture D is the best performing mixture of the oil based resin silane system in terms of pull out force and rubber coverage. It contains hydrolyzed A1289 and A1170. Stoichiometric quantity of water was added to just hydrolyze the A1289. Acetone was added in equal parts to water.

Drying had a positive effect on mixture B, no effect on mixture C and a negative effect on mixture D in terms of the pull out force values. However, rubber coverage dropped drastically as a result of drying for the oil based resin silane mixtures.

With respect to the oil based WD 510 resin silane system, the combination of cleaning and not drying gave the best adhesion value. Drying decreases the pull out force by 18% and increases the rubber coverage by almost 50% for this system.

Based on this testing, cleaning affects the pull out value positively. However, higher silane concentrations not only gave lower pull out values, but cleaning had little or no effect on the adhesion values. Lower silane concentrations gave the best adhesion values. For sample #1, cleaning improved the adhesion value by 190%.

Those samples that were not cleaned had 0% rubber coverage. However, among the cleaned samples, silane mixture #1 gave the maximum coverage. The rubber coverage dropped off at higher silane concentrations.

The effect of cleaning on the performance of the oil based resin silane mixture was also tested. The below listed values are measured on a 100g total weight basis. A 1:3 ratio was maintained between A1170 and A1289. Mixtures I, III and V have equal parts resin and A1170. Mixtures II, IV and VI have equal parts resin and the total silane concentration. The wires were cleaned as described and were then coated with the below silane mixtures. The uncleaned wires were also coated with these silane mixtures. These wires were then cured in the rubber compound and tested under tension for adhesion.

**Table 4**

| **Constituents of the different oil based WD 510 resin silane mixture** | | | | | | | |
|---|---|---|---|---|---|---|---|
| Silane mixture | Silane concentration (%) | A1170 (g) | A1289 (g) | Resin WD 510 (g) | Lubricant (9) | Cleaned Pullout Force (kg) | Uncleaned Pullout Force (kg) |
| I | 1 | 0.25 | 0.75 | 0.25 | 98.75 | 29.3 | 10.2 |
| II | 1 | 0.25 | 0.75 | 1.0 | 98 | 25.8 | 11.5 |
| III | 5 | 1.25 | 3.75 | 1.25 | 93.75 | 27.3 | 10.3 |
| IV | 5 | 1.25 | 3.75 | 5.0 | 90 | 16.3 | 13 |
| V | 5 | 1.25 | 3.75 | 5.0 | 90 | 17 | 17.6 |
| VI | 20 | 5 | 15 | 20 | 60 | 12 | 13.9 |
| Control | | | | | | 12 | 11.3 |

To assess the difference in performance between the oil based neat and hydrolyzed silane resin mixture, the formulations in Table 5 and Table 6 were tested.

**Table 5**

| **Oil based neat silane-resin system** | | | | | | |
|---|---|---|---|---|---|---|
| Silane mixture | Silane concentration (%) | A1170 (g) | A1289 (g) | Resin WD 510 (g) | Lubricant (g) | Pullout Force (kg) |
| 1 | 1 | 0.25 | 0.75 | 0.25 | 98.75 | 29.3 |
| 2 | 1 | 0.25 | 0.75 | 1.0 | 98 | 25.8 |
| 3 | 5 | 1.25 | 3.75 | 1.25. | 93.75 | 27.3 |
| 4 | 5 | 1.25 | 3.75 | 5.0 | 90 | 16.3 |
| 5 | 10 | 2.5 | 7.5 | 2.5 | 87.5 | 17.6 |
| 6 | 10 | 2.5 | 7.5 | 10 | 80 | 13.9 |
| 7 | 20 | 5.0 | 15 | 5 | 75 | 16.4 |
| 8 | 20 | 5.0 | 15 | 20 | 60 | 15.7 |

**Table 6**

| **Oil based hydrolyzed silane-resin system** | | | | | | |
|---|---|---|---|---|---|---|
| Silane mixture | Silane concentration (%) | A1170 (10% soln) (g) | A1289 (62.5% soln) (g) | Resin WD 510 (g) | Lubricant (g) | Pullout Force (kg) |
| 1H | 1 | 2.5 | 1.2 | 0.25 | 96.5 | 21.5 |
| 2H | 1 | 2.5 | 1.2 | 1 | 95.3 | 19.7 |
| 3H | 5 | 12.5 | 6.0 | 1.25 | 80.25 | 25.8 |
| 4H | 5 | 12.5 | 6.0 | 5 | 76.5 | 24.2 |
| 5H | 10 | 25 | 12 | 2.5 | 60.5 | 10.7 |
| 6H | 10 | 25 | 12 | 10 | 53 | N/A |
| 7H | 20 | 50 | 24.2 | 5 | 20.8 | 15.6 |
| 8H | 20 | 50 | 24.2 | 20 | 5.8 | N/A |

The cleaned wires were coated with the above silane mixtures and cured in the rubber compound and later tested in tension for adhesion.

Hydrolyzed mixtures 6 and 8 gelled when the respective components were mixed. As such, they were not tested.

Neat silanes performed better than hydrolyzed silanes except for mixture #4 where the hydrolyzed silane outperformed the neat silane by 50% with respect to pull out force. Silane mixture #1 was the best performer among the 16 different solutions. Among the hydrolyzed solutions, mixture #3 was the top performer.

To determine the effect of varying the ratio and concentration of neat and hydrolyzed silanes on the pull out values, the formulations shown in Table 7 and Table 8 were tested.

**Table 7**

| **Oil based neat silane-resin system** | | | | | | |
|---|---|---|---|---|---|---|
| Silane mixture | Silane ratio | Silane concentration (%) | A1170 (g) | A1289 (g) | Resin WD 510 (g) | Lubricant (g) |
| I | 1:1 | 1 | 0.5 | 0.5 | 0.5 | 98.5 |
| J | 1:3 | 1 | 0.25 | 0.75 | 0.25 | 98.75 |
| K | 1:5 | 1 | 0.166 | 0.833 | 0.16 | 98.83 |
| L | 1:1 | 5 | 2.5 | 2.5 | 2.5 | 92.5 |
| M | 1:3 | 5 | 1.25 | 3.75 | 1.25 | 93.75 |
| N | 1:5 | 5 | 0.83 | 4.15 | 0.83 | 94.19 |

**Table 8**

| **Oil based hydrolyzed silane-resin system** | | | | | | |
|---|---|---|---|---|---|---|
| Silane mixture | Silane ratio | Silane concentration (%) | A1170 (10% soln) (g) | A1289 (62.5% soin) (g) | Resin WD 510 (g) | Lubricant (g) |
| O | 1:1 | 1 | 5.0 | 0.8 | 0.5 | 93.7 |
| P | 1:3 | 1 | 2.5 | 1.20 | 0.25 | 96.05 |
| Q | 1:5 | 1 | 1.66 | 1.34 | 0.16 | 96.84 |
| R | 1:1 | 5 | 25 | 4.03 | 2.5 | 68.47 |
| S | 1:3 | 5 | 12.5 | 6.04 | 1.25 | 80.21 |
| T | 1:5 | 5 | 8.3 | 6.69 | 0.83 | 84.18 |

Control, hydrolyzed mixture #6 and hydrolyzed mixture #8 have zero rubber coverage. Highest rubber coverage is offered by both neat and hydrolyzed silane mixture #1. In other cases, neat silane mixtures offer more rubber coverage except in mixture #7 where the hydrolyzed mixture offers 125% more coverage than the neat solution.

An analysis of line speed to drying temperature indicated that maximum pull out force was achieved at about 4m/min with a drying temperature of 140°C.

Thus, as shown, the present invention permits the application of a wide variety of different silane formulations onto metal surfaces using an oil. The applied silanes then function to improve adhesion and provide other attributes typically associated with a silane coating, such as corrosion inhibition. Applying the silane coating with an oil bath provides greater flexibility in applying the silane, allowing it to be incorporated in line with many different processes. Many different processes require an oil coating, therefore the application of silane can be accomplished without additional equipment. This is particularly the case when the metal being coated is tire cord. In such an application, the applied silane coating significantly improves the adhesion of the sulfur cured rubber to the tire cord while at the same time permitting the use of a rubber formulation that does not include a cobalt compound and has lower levels of sulfur, thereby improving the overall physical characteristics of the rubber itself.

This has been a description of the present invention along with the preferred method of practicing the present invention.

## Claims

1. A method of applying a silane coating onto a metal substrate comprising contacting said metal substrate with an oil mixture, wherein said oil mixture comprises at least 80% by weight oil and 0.5 to 10% organofunctional silane by weight, and wherein the oil is selected from the group comprising naphthenic lubricating oils, paraffinic lubricating oils, animal based lubricating oils, vegetable based lubricating oils and synthetic lubricants comprisng polyglycols, dibasic acid esters, chlorofluorocarbons, silicone oils, neopentyl polyol esters and polyphenyl ethers.

2. The method claimed in claim 1 wherein said metal substrate is wire and said wire is drawn through said oil mixture.

3. The method claimed in claim 2 wherein said organofunctional silane is dispersed in a resin.

4. The method claimed in claim 1 wherein said silane includes an amino silane.

5. The method claimed in claim 1 wherein said organofunctional silane comprises at least 2% by weight of said oil mixture.

6. The method claimed in claim 1 wherein said organofunctional silane is a mixture amino silane and polysulfur silane.

7. The method claimed in claim 6 wherein said organofunctional silane mixture has a ratio by weight of amino silane:polysulfur silane of 1:3 to 3:1.

8. The method claimed in claim 2 wherein said wire is maintained in said bath for a period of at least 1 second.

9. The method claimed in claim 1 wherein said organofunctional silane is unhydrolyzed.

10. The method claimed in claim 1 wherein said organofunctional silane is hydrolyzed and said solution further includes water.

11. The method claimed in claim 1 wherein said oil is a naphthenic lubricating oil.

12. The method claimed in claim 1 wherein said oil is a paraffinic lubricating oil.

13. The method claimed in claim 1 wherein said metal substrate is cleaned with an alkaline cleaner before said silane is applied.

14. A coating composition comprising at least 80% by weight oil and 0.5% to 10% organofunctional silane by weight, and wherein the oil is selected from the group comprising naphthenic lubricating oils, paraffinic lubricating oils,animal based lubricating oils, vegetable based lubricating oils and synthetic lubricants comprising polyglycols, dibasic acid esters, chlorofluorocarbons, silicone oils, neopentyl polyol esters and polyphenyl ethers.

15. The composition claimed in claim 14 wherein oil comprises at least 90% by weight of said composition.

16. The composition claimed in claim 14 wherein said organofunctional silane comprises a mixture of amino silane and polysulfur silane.

17. The composition claimed in claim 14 wherein said organofunctional silane is unhydrolyzed.

18. The composition claimed in claim 14 wherein said composition further includes a resin dispersible in said oil.

19. The composition claimed in claim 18 wherein said resin comprises an epoxy.

20. The composition claimed in claim 14 wherein said oil is a naphthenic oil.

## Patentansprüche

1. Verfahren zum Applizieren einer Silanbeschichtung auf ein Metallsubstrat, das das Inkontaktbringen des genannten Metallsubstrats mit einem Ölgemisch beinhaltet, wobei das genannte Ölgemisch wenigstens 80 Gew.-% Öl und 0,5 bis 10 Gew.-% organofunktionelles Silan umfasst und wobei das Öl ausgewählt wird aus der Gruppe bestehend aus naphthenischen Schmierölen, paraffinischen Schmierölen, Schmierölen auf tierischer Basis, Schmierölen auf pflanzlicher Basis und synthetischen Schmiermitteln, die Polyglykole, dibasische Säureester, Fluorchlorkohlenwasserstoffe, Silikonöle, Neopentyl-Polyolester und Polyphenylether umfassen.

2. Verfahren nach Anspruch 1, wobei das genannte Metallsubstrat Draht ist und der genannte Draht durch das genannte Ölgemisch gezogen wird.

3. Verfahren nach Anspruch 2, wobei das genannte organofunktionelle Silan in einem Harz dispergiert ist.

4. Verfahren nach Anspruch 1, wobei das genannte Silan ein Aminosilan beinhaltet.

5. Verfahren nach Anspruch 1, wobei das genannte organofunktionelle Silan wenigstens 2 Gew.-% des genannten Ölgemischs umfasst.

6. Verfahren nach Anspruch 1, wobei das genannte organofunktionelle Silan ein Gemisch aus Aminosilan und Polyschwefelsilan ist.

7. Verfahren nach Anspruch 6, wobei das genannte organofunktionelle Silangemisch ein Gewichtsverhältnis von Aminosilan zu Polyschwefelsilan von 1:3 bis 3:1 hat.

8. Verfahren nach Anspruch 2, wobei der genannte Draht für eine Periode von wenigstens 1 Sekunde in dem genannten Bad gehalten wird.

9. Verfahren nach Anspruch 1, wobei das genannte organofunktionelle Silan unhydrolysiert ist.

10. Verfahren nach Anspruch 1, wobei das genannte organofunktionelle Silan hydrolysiert ist und die genannte Lösung ferner Wasser beinhaltet.

11. Verfahren nach Anspruch 1, wobei das genannte Öl ein naphthenisches Schmieröl ist.

12. Verfahren nach Anspruch 1, wobei das genannte Öl ein paraffinisches Schmieröl ist.

13. Verfahren nach Anspruch 1, wobei das genannte Metallsubstrat mit einem alkalischen Reiniger gereinigt wird, bevor das genannte Silan aufgebracht wird.

14. Beschichtungszusammensetzung, die wenigstens 80 Gew.-% Öl und 0,5 bis 10 Gew.-% organofunktionelles Silan umfasst und wobei das Öl ausgewählt ist aus der Gruppe bestehend aus naphthenischen Schmierölen, paraffinischen Schmierölen, Schmierölen auf tierischer Basis, Schmierölen auf pflanzlicher Basis und synthetischen Schmiermitteln, die Polyglykole, dibasische Säureester, Fluorchlorkohlenwasserstoffe, Silikonöle, Neopentyl-Polyolester und Polyphenylether umfassen.

15. Zusammensetzung nach Anspruch 14, wobei Öl wenigstens 90 Gew.-% der genannten Zusammensetzung ausmacht.

16. Zusammensetzung nach Anspruch 14, wobei das genannte organofunktionelle Silan ein Gemisch aus Aminosilan und Polyschwefelsilan umfasst.

17. Zusammensetzung nach Anspruch 14, wobei das genannte organofunktionelle Silan unhydrolysiert ist.

18. Zusammensetzung nach Anspruch 14, wobei die genannte Zusammensetzung ferner ein in dem genannten Öl dispergierbares Harz ist.

19. Zusammensetzung nach Anspruch 18, wobei das genannte Harz ein Epoxid umfasst.

20. Zusammensetzung nach Anspruch 14, wobei das genannte Öl ein naphthenisches Öl ist.

## Revendications

1. Procédé d'application d'un revêtement de silane sur un substrat métallique, comprenant mettre ledit substrat métallique en contact avec un mélange d'huile, où ledit mélange d'huile comprend au moins 80 % en poids d'huile et de 0,5 à 10 % en poids de silane organofonctionnel, et où l'huile est sélectionnée parmi le groupe consistant en huiles lubrifiantes naphténiques, huiles lubrifiantes paraffiniques, huiles lubrifiantes de base animale, huiles lubrifiantes de base végétale et lubrifiants synthétiques comprenant des polyglycols, esters d'acide dibasique, chlorofluorocarbones, huiles de silicone, esters de polyol de néopentyle et éthers de polyphényle.

2. Procédé selon la revendication 1, où ledit substrat métallique est du fil métallique et ledit fil métallique est tiré à travers ledit mélange d'huile.

3. Procédé selon la revendication 2, où ledit silane organofonctionnel est dispersé dans une résine.

4. Procédé selon la revendication 1, où ledit silane comprend un aminosilane.

5. Procédé selon la revendication 1, où ledit silane organofonctionnel comprend au moins 2 % en poids dudit mélange d'huile.

6. Procédé selon la revendication 1, où ledit silane organofonctionnel est un mélange d'aminosilane et de silane polysulfuré.

7. Procédé selon la revendication 6, où ledit mélange de silane organofonctionnel a un rapport en poids d'aminosilane:silane polysulfuré de 1:3 à 3:1.

8. Procédé selon la revendication 2, où ledit fil métallique est maintenu dans ledit bain pendant une période de 1 seconde au moins.

9. Procédé selon la revendication 1, où ledit silane organofonctionnel est non hydrolysé.

10. Procédé selon la revendication 1, où ledit silane organofonctionnel est hydrolysé et ladite solution comprend en outre de l'eau.

11. Procédé selon la revendication 1, où ladite huile est une huile lubrifiante naphténique.

12. Procédé selon la revendication 1, où ladite huile est une huile lubrifiante paraffinique.

13. Procédé selon la revendication 1, où ledit substrat métallique est nettoyé avec un agent de nettoyage alcalin préalablement à l'application du silane.

14. Composition de revêtement comprenant au moins 80 % en poids d'huile et de 0,5 à 10 % en poids de silane organofonctionnel, et où l'huile est sélectionnée parmi le groupe consistant en huiles lubrifiantes naphténiques, huiles lubrifiantes paraffiniques, huiles lubrifiantes de base animale, huiles lubrifiantes de base végétale et lubrifiants synthétiques comprenant des polyglycols, esters d'acide dibasique, chlorofluorocarbones, huiles de silicone, esters de néopentyl polyols et éthers de polyphényle.

15. Composition selon la revendication 14, dans laquelle l'huile comprend au moins 90 % en poids de ladite composition.

16. Composition selon la revendication 14, dans laquelle ledit silane organofonctionnel comprend un mélange d'aminosilane et de silane polysulfuré.

17. Composition selon la revendication 14, dans laquelle ledit silane organofonctionnel est non hydrolysé.

18. Composition selon la revendication 14, où ladite composition comprend en outre une résine dispersible dans ladite huile.

19. Composition selon la revendication 18, dans laquelle ladite résine comprend une époxy.

20. Composition selon la revendication 14, dans laquelle ladite huile est une huile naphténique.
